

# UNITED STATES PATENT OFFICE.

WALTER I. OESCHGER, OF DETROIT, MICHIGAN, ASSIGNOR TO PARKER RUST PROOF COMPANY OF AMERICA, OF DETROIT, MICHIGAN, A CORPORATION OF MICHIGAN.

## PROCESS FOR RUST-PROOFING IRON AND STEEL.

1,254,264.

Specification of Letters Patent.

Patented Jan. 22, 1918.

No Drawing.

Application filed February 21, 1917. Serial No. 150,016.

To all whom it may concern:

Be it known that I, WALTER I. OESCHGER, a citizen of the United States, and residing at Detroit, in the county of Wayne and 5 State of Michigan, have invented a new and Improved Process for Rust-Proofing Iron and Steel, of which the following is a specification.

This invention relates to a process for 10 forming rust-proof surfaces on articles of iron and steel or alloys thereof, and its object is to provide a process whereby the articles to be treated are subjected to fumes or vapors which produce surfaces of basic fer- 15 ro-ferric phosphates of iron which are heavy and very dense.

This invention consists in subjecting the 20 surfaces of the articles of iron and steel to be treated to fumes or vapors produced by highly heating metallic phosphates such as the acid meta-phosphates of tungsten, molybdenum or of any of the metals of the third, fourth and fifth groups, according to 25 the analytical classification (set forth by Prof. G. S. Newth, F. I. C., F. C. S., in the eighth edition of his "Manual of Chemical Analysis," published by Longmans, Green & Co., New York, in 1909), either singly or in combination with each other.

30 In this classification, tungsten is in the first group, molybdenum in the second group, while the third, fourth and fifth groups include aluminum, chromium, cobalt, iron, nickel, manganese, zinc, barium, 35 strontium, calcium, sodium, potassium, magnesium and vanadium.

The acid meta-phosphate of most general 40 application is made by placing a quantity of iron oxid, preferably powdered black iron scale,  $(Fe_3O_4)$  in a pot with sufficient phosphoric acid to form a soft paste. A quantity of water about equal in amount to the acid may be added to keep the mass from caking, after which heat is applied and the 45 material is stirred until a dry granular mass is obtained, which is then powdered. The

acid and oxid may be heated before the water is added if desired.

The reactions may be expressed as follows:—When heated

50



And continued heating results in driving off the water of combination

55



This is an acid meta-phosphate.

Carbonates and oxids of the other metals 60 may be similarly treated. Care must be taken to avoid heating these phosphates to a point where there is more than merely perceptible fuming.

The articles to be treated are preferably 65 previously heated to about 600 degrees F. in order to obtain the best results. While cold metal may be treated with satisfactory final results by this process, the time required is very great. When heated to the 70 temperature indicated, the articles can be rendered rust-proof in from ten to forty minutes. The articles may be treated in the furnace wherein they are heated or they may be placed in a special treating chamber.

75

The acid meta-phosphates are heated to a high temperature to produce abundant fumes which are acid in character. This may be done in the treating chamber or in an especially constructed furnace, the 80 fumes being drawn into the treating chamber by means of a suction fan placed where most effective. If desired, a jet of dry steam may be caused to enter the treating chamber to render the fumes more active in 85 character. The duration of the treatment will depend upon the character of the metals treated and also upon the desired character of the coating.

It has been found that the mixing of 90 about two per cent. of the acid meta-phosphates of molybdenum, strontium or

tungsten with the iron acid meta-phosphates intensifies the action of the fumes and renders them especially effective for high carbon steels. There is little advantage in using these acid meta-phosphates of the rarer metals alone or in combination with each other, or in using more than two per cent in combination with iron acid meta-phosphate.

10 After the fuming, vapors of oil may be carried into contact with the surfaces treated or the articles may be sprayed with or dipped into the oil. The surfaces of basic iron phosphates are admirably adapted to receive paint, enamel, lacquer and even other metals by electro-plating.

15 Volatile metals such as zinc may be mixed with the acid meta-phosphates during the time they are heated to produce the fumes, and the action thereof seems to be the production of more even and dense surfaces having high resistance to the corroding effects of the elements in the atmosphere.

20 The combination of molybdenum, tungsten or any of the metals of the third, fourth and fifth groups as stated above, with an excess of meta-phosphoric acid to form a paste is temporary and may be partly broken up at any time by the application of 25 heat. These metals all have the characteristic of freely entering into this combination. The fumes are produced by the decomposition of these acid salts, and are delivered more regularly than if the meta-phosphoric acid is heated alone, probably owing to the mechanical carrying over of 30 small particles of acid when the liquid boils.

35 I claim:—

1. A new and useful process consisting in 40 subjecting articles of iron and steel to the action of fumes from acid meta-phosphates of tungsten, molybdenum or of any of the metals of the third, fourth and fifth groups, singly or in combination with each other.
2. A new and useful process consisting in 45 subjecting articles of iron and steel to the action of steam mixed with the fumes from

acid meta-phosphates of tungsten, molybdenum or of any of the metals of the third, fourth and fifth groups.

50

3. A new and useful process consisting in subjecting heated articles of iron and steel to the action of fumes caused by heating acid meta-phosphates of tungsten, molybdenum or of any of the metals of the third, fourth and fifth groups.

55

4. A new and useful process consisting in subjecting articles of iron and steel to the action of fumes produced by heating acid meta-phosphates of tungsten, molybdenum, 60 or of any of the metals of the third, fourth and fifth groups either alone or in combination with each other.

65

5. A new and useful process consisting in subjecting articles of iron and steel to the action of fumes produced by heating acid meta-phosphates of iron.

70

6. A new and useful process consisting in subjecting articles of iron and steel to the action of fumes produced by heating acid meta-phosphates of iron mixed with a small percentage of acid meta-phosphate of molybdenum, strontium or tungsten.

75

7. A new and useful process consisting in subjecting heated articles of iron and steel to the action of fumes produced by heating acid meta-phosphates of iron to which fumes a quantity of steam has been added.

80

8. A new and useful process consisting in subjecting articles of iron and steel to the action of fumes produced by heating acid meta-phosphates of iron, to which fumes a quantity of steam has been added.

85

9. A new and useful process consisting in subjecting articles of iron and steel to the action of fumes produced by heating acid meta-phosphates of iron and a volatile metal.

90

10. A new and useful process consisting in subjecting articles of iron and steel to the action of fumes produced by heating acid meta-phosphates of iron and zinc.

WALTER I. OESCHGER.